

# UNITED STATES PATENT OFFICE.

BOTHO SCHWERIN, OF FRANKFORT-ON-THE-MAIN, GERMANY, ASSIGNOR TO GESELLSCHAFT FÜR ELEKTRO-OSMOSE M. B. H., OF FRANKFORT-ON-THE-MAIN, GERMANY, A CORPORATION.

## PROCESS TO LOWER THE VITRIFYING-POINT OF CERAMIC SUBSTANCES.

1,121,408.

Specification of Letters Patent. Patented Dec. 15, 1914.

No Drawing.

Application filed February 27, 1913. Serial No. 751,140.

To all whom it may concern:

Be it known that I, Botho Schwerin, a subject of the German Emperor, residing at Frankfort-on-the-Main, Germany, have invented certain new and useful Improvements in Processes to Lower the Vitrifying-Point of Ceramic Substances, of which the following is a specification.

There are certain materials, such as soap-stone, steatite and other similar silicates of magnesia, which deform and vitrify at approximately the same temperature and any attempt to fire objects formed of these materials after the materials have been finely ground is found impracticable, for the reason that the material forming the objects does not vitrify or become dense before deforming and the objects do not keep their form after the deformation has begun. To overcome this difficulty, it has been the usual practice to lower the vitrifying points of the above-named materials by the addition of kaolin and similar substances which, in conjunction with the original material, forms a composition which vitrifies at a lower temperature. This practice is attended with the lowering of the vitrifying point, so that it is possible to preserve the form of the objects, inasmuch as the same do not deform, but on the other hand, these objects naturally have the drawback of not being composed entirely of the pure, original material. It is found that objects so prepared have lost more or less of their former characteristics possessed before the addition of the binding material. This drawback has many different effects among which may be mentioned, for instance, the loss of insulation capacity, the loss of elasticity and the loss of solidity. The present invention seeks to provide a process which shall result in a finished product free from the faults just mentioned.

It is the object of the present invention to provide a process by the practice of which the vitrifying point of such substances as soap-stone, steatite, and similar silicates of magnesia may be lowered preparatory to burning, so as to make it possible to burn said articles from the pure material without any foreign substance being mixed therewith.

The method of procedure in the present invention is as follows: The raw material is

finely ground and purified, and a suitable amount thereof is then suspended in water to which is added or has previously been added, a proportionate amount of a suitable electrolyte, for instance, for each kilogram of dry steatite one gram of sodium silicate may be added. The finest particles thereby get into sol-condition in a manner disclosed in my United States Patent No. 1,029,579, the coarser particles and what foreign matter may be present settling. After a given time determined according to the amount or degree by which it is desired to lower the sintering point of the materials, the suspension is drawn off, put in an electro-osmotic machine and exposed to the action of an electric current whereby the material is deposited on the anode in relatively dry form, as set forth in my United States Patent No. 993,888. The deposited material is then taken from the anode and mixed with the necessary amount of water for the forming or casting of objects, after which the objects may be burned in the well-known manner.

The results of the process just set forth will be described in connection with the following table:

| No. 1.<br>Seger cone. | No. 2.<br>Degrees<br>centigrade. | Percentage of water absorbed. |                                         |                                          | 85 |
|-----------------------|----------------------------------|-------------------------------|-----------------------------------------|------------------------------------------|----|
|                       |                                  | No. 3.<br>Untreated.          | No. 4. Af-<br>ter standing<br>72 hours. | No. 5. Af-<br>ter standing<br>120 hours. |    |
| 01                    | 900                              | 15.36                         | 26.62                                   | 20.0                                     | 90 |
| 5                     | 1150                             | 17.91                         | 16.05                                   | 0.022                                    |    |
| 9                     | 1250                             | 14.13                         | 6.36                                    | 0.001                                    |    |
| 12                    | 1350                             | 12.55                         | 0.001                                   | 0.0                                      |    |
| 14                    | 1410                             | 11.11                         | 0.002                                   | 0.0                                      |    |
| 16                    | 1460                             | 9.58                          | 0.001                                   | 0.0                                      |    |
| 18                    | 1500                             | 7.54                          | 0.0                                     | 0.0                                      |    |
| 20                    | 1550                             | Melts.                        | Melts.                                  | Melts.                                   |    |

95

The first column of the table represents the number of the cone in the series of Seger cones, the deformation point of which agrees with the temperatures opposite in the second column. Column 2 indicates the temperature on a centigrade scale corresponding to the Seger cones. Columns 4 and 5 represent the percentages of water absorbed by specimens made according to the present invention, whereas column 3 indicates the percentage of water absorbed by the original material which had been formed ready for the burning without having been sub-

100

105

jected to the process disclosed herein. Referring to column 3, it will be seen that objects made from the pure, untreated material, which in this instance was steatite, will 5 absorb water irrespective of the temperature at which they are burned, except at the temperature of 1530°, at which temperature objects deform. The fourth column shows the 10 percentage of water absorbed by specimens made from the material treated according to the present invention where the particles were in suspension for 72 hours before being collected. It will be noted that the specimen 15 which was burned at a temperature of 1350° centigrade absorbed 4/1000 of 1% of water, whereas the specimen made from the untreated material at the same temperature absorbed 12.55% water. The fifth column shows the 20 percentage of water absorbed by specimens which were made from material treated according to the present invention where the material before collection in the electro-osmotic machine had stood for 120 hours. It will be seen that the specimen so 25 made, which was burned at the temperature of 1350° centigrade had zero absorption of water. See column 5. It will further be noted that specimens made from materials treated according to the present invention 30 could be burned without deforming at such a temperature that the burning would prevent absorption of water. Thus the materials shown in the 4th and 5th columns when burned at 1500° centigrade had zero as a 35 water absorption. It will further be noted that at 1530° centigrade the material deformed so that the deformation point is not affected by the present process but the vitrification point is affected. 40 It will be understood that the vitrifying referred to herein is a partial melting, though not a complete melting, whereby the particles forming the objects stick together in such a way as to make the article dense, 45 the higher the degree of vitrification the more dense the object and therefore the more impervious to water. For this reason, the percentage of water absorption can be taken to indicate in an approximate manner the 50 degree of vitrification. Whatever be the relation between the percentage of water ab-

sorption and the degree of vitrification before the water absorption becomes zero, is of little consequence, the important point to be borne in mind being that when the percentage of water absorption has reached zero, the material has been perfectly vitrified. Thus is it seen that the lowering of the vitrifying point depends upon the fineness of the particles in the sol-condition 55 which are collected and from which the objects to be burned are formed. However, it is found that the vitrifying point also depends upon the nature of the electrolyte through the addition of which the matter in suspension is brought into a sol-condition. For instance, the vitrifying point will be lowered less when ammonia is used as an electrolyte than when either sodium hydroxid or sodium silicate is used as the 60 electrolyte. With equal settling duration, the vitrifying point of the same material can be lowered more or less through the addition of an electrolyte of more or less activity. 75

I claim:

1. The process of making ceramics having a desired degree of water absorption from a substance which untreated deforms at the temperature of true vitrification which consists in powdering the original substance, suspending the same, bringing the same in sol-condition, permitting the solution to stand for an interval of time, collecting the said particles from the suspension and sintering the same. 80

2. The process of preparing for burning, material having a desired degree of water absorption from a substance which untreated deforms at the temperature of true vitrification which consists in powdering the material, suspending the same, bringing the substance into sol-condition, permitting said substance to stand an interval of time, and collecting the particles in suspension. 90

In testimony whereof I affix my signature in presence of two witnesses.

BOTHO SCHWERIN.

Witnesses:

JEAN GRUND,  
CARL GRUND.